# EUROPEAN PATENT SPECIFICATION

(11) **EP 3 395 978 B1**
(45) Date of publication and mention of the grant of the patent: **16.12.2020**
(21) Application number: 16879340.4
(22) Date of filing: 21.12.2016
(51) Int. Cl.: C22C 38/00, C22C 38/04, C22C 38/14, C21D 9/46, C21D 8/02, C21D 6/00, C22C 38/02, C22C 38/08, C22C 38/12, C22C 38/38

(54) **HIGH MANGANESE STEEL SHEET HAVING EXCELLENT VIBRATION-PROOF PROPERTY, AND MANUFACTURING METHOD THEREFOR**
STAHLBLECH MIT HOHEM MANGANGEHALT UND HERVORRAGENDER VIBRATIONSBESTÄNDIGKEIT UND HERSTELLUNGSVERFAHREN DAFÜR
TÔLE D'ACIER À HAUTE TENEUR EN MANGANÈSE AYANT UNE EXCELLENTE PROPRIÉTÉ D'AMORTISSEMENT DES VIBRATIONS ET PROCÉDÉ DE FABRICATION S'Y RAPPORTANT

(30) Priority: 23.12.2015 KR 20150185471
(43) Date of publication of application: 31.10.2018
(73) Proprietor: Posco, Pohang-si, Gyeongsangbuk-do 37859 (KR)
(72) Inventor: CHO, Won-Tae, Gwangyang-si Jeollanam-do 57807 (KR); KIM, Tai-Ho, Gwangyang-si Jeollanam-do 57807 (KR); CHIN, Kwang-Geun, Gwangyang-si Jeollanam-do 57807 (KR); KIM, Young-Ha, Gwangyang-si Jeollanam-do 57807 (KR); SONG, Tae-Jin, Gwangyang-si Jeollanam-do 57807 (KR)
(74) Representative: Zech, Stefan Markus
(86) International application number: PCT/KR2016/015040
(87) International publication number: WO 2017/111473

(56) References cited:
- EP-A1- 2 778 247
- EP-A2- 0 649 914
- WO-A1-2006/109919
- WO-A1-2015/060499
- CN-A- 103 898 401
- JP-A- 2004 137 579
- JP-A- 2007 126 715
- JP-A- 2011 230 182
- KR-A- 20140 085 225
- KR-A- 20140 119 216
- KR-A- 20150 074 974
- KR-B1- 100 840 287
- US-A- 5 891 388

## Description

### [Technical Field]

The present disclosure relates to a high Mn steel sheet having excellent damping properties, provided as a steel sheet for a vehicle or construction equipment and used in a location requiring damping properties for noise reduction.

### [Background Art]

In recent years, noise reduction in vehicle manufacturing and building materials is a problem which manufacturers have needed to solve. In the case of vehicle manufacturers, it is particularly necessary to have damping properties in addition to excellent mechanical properties in components such as engine parts, oil pans, and the like, in which a significant noise is generated. In the case of building materials, recently, due to the strengthening of regulations relating to noise between floors, the development of a damping steel sheet as a floor plate of a duplex building including an apartment building is required.

High Mn damping steel is steel having good damping properties and excellent mechanical properties, since noise energy may be converted to thermal energy due to interface sliding of epsilon martensite when an external impact is applied.
Patent Document EP 2 778 247 A1 relates to steel sheet for warm press forming, the steel sheet comprising, by weight%, C: 0.01% to 0.5%, Si: 3.0% or less (excluding 0%), Mn: 3% to 15%, P: 0.0001% to 0.1%, S: 0.0001% to 0.03%, A1 3.0% or less (excluding 0%), N: 0.03% or less (excluding 0%), and the balance of Fe and inevitable impurities.
Patent Document WO 2015/060499 A1 relates to a high-strength and high-manganese steel sheet suitable for an outer panel or a vehicle body of a transport vehicle and, more specifically, to a high-strength and high-manganese steel sheet having excellent vibration-proof properties and a method for producing the same.

### [Disclosure]

### [Technical Problem]

An aspect of the present disclosure may provide a high Mn steel sheet having excellent damping properties and a method for manufacturing the same.

### [Technical Solution]

According to an aspect of the present disclosure, a high Mn steel sheet, having excellent damping properties, includes: 0 wt% to 0.1 wt% of carbon (C), 8 wt% to 30 wt% of manganese (Mn), 0.1 wt% or less of phosphorus (P), 0.02 wt% or less of sulfur (S), 0.1 wt% or less of nitrogen (N), 0 wt% to 1.0 wt% of titanium (Ti), the balance of Fe and inevitable impurities, the high Mn steel sheet further optionally comprising one, two, or more among 0 wt% to 3 wt% of silicon (Si), 0.005 wt% to 5.0 wt% of chromium (Cr), 0.005 wt% to 2.0 wt% of nickel (Ni), 0.005 wt% to 0.5 wt% of niobium (Nb), 0.0001 wt% to 0.01 wt% of boron (B), 0.005 wt% to 0.5 wt% of vanadium (V), and 0.005 wt% to 1 wt% of tungsten (W), a microstructure of the steel sheet consist of epsilon martensite and austenite, and an average particle diameter of each of the epsilon martensite and the austenite is 2 µm or less.

### [Advantageous Effects]

According to an exemplary embodiment in the present disclosure, a high Mn steel sheet having excellent damping properties is provided, and is used for structural components for a vehicle and building materials such as a flooring material, in which a noise reduction is required.

### [Description of Drawings]

FIG. 1 is a view illustrating the microstructures of the Example heat treated at 600°C and the Comparative Example heat treated at 800°C to 1000°C.
FIG. 2 is a drawing illustrating a dilatometer cycle of the heat treatment illustrated in FIG. 1.
FIG. 3 is a graph illustrating the results of specific damping capacity (SDC) measured by the internal resistance method with respect to the Example and the Comparative Example (4).

### [Best Mode for Invention]

Hereinafter, the present disclosure will be described in detail.

The present disclosure relates to a high Mn steel sheet having excellent damping properties and a method for manufacturing the same. The high Mn steel sheet includes 0 wt% to 0.1 wt% or less of carbon (C), 8 wt% to 30 wt% of manganese (Mn), 0.1 wt% or less (including 0%) of phosphorus (P), 0.02 wt% or less (including 0%) of sulfur (S), 0.1 wt% or less (including 0%) of nitrogen (N), 0 wt% to 1.0 wt% (excluding 0%) of titanium (Ti), and iron (Fe) and inevitable impurities. A microstructure of the steel sheet consists of epsilon martensite and austenite, and an average particle diameter of each of the epsilon martensite and the austenite is 2 µm or less.

A specific steel composition of the steel sheet according to the present disclosure and the reasons for restricting the steel composition thereof are as follows.

If the addition amount of carbon (C) exceeds 0.1%, carbides may be excessively precipitated, and the hot workability and elongation are lowered, and the damping capability may be significantly reduced. Thus, the addition amount of C is limited to 0.1% or less.

Manganese (Mn) is an element essential for stably securing an austenite structure and is an element for increasing the stacking fault energy. If an addition amount of Mn is less than 8%, martensite, degrading formability, is formed. Thus, strength increases but ductility significantly decreases. Moreover, the stacking fault energy is lowered, so austenite, partially formed, may be easily transformed into epsilon martensite. Thus, a lower limit of Mn is limited to 8%. On the other hand, if the addition amount of Mn exceeds 30%, manufacturing costs may be increased due to a large amount of Mn, and slab cracking may be caused by an increase in an amount of phosphorus (P) in steel. Moreover, as the addition amount of Mn increases, internal grain boundary oxidation significantly occurs when a slab is reheated. Thus, an oxide defect on a surface of a steel sheet is caused. Moreover, surface properties are degraded in hot dip galvanizing. Thus, an upper limit of the addition amount of Mn is limited to 30%.

Phosphorus (P) and sulfur (S) are inevitably included when steel is produced. The content of P is limited to 0.1% or less (including 0%), and the content of S is limited to 0.02% or less (including 0%). In detail, in the case of P, segregation occurs, so the workability of steel may be reduced. In the case of S, coarse manganese sulfide (MnS) is formed, so a defect such as flange cracking may be generated, and the hole expansion of a steel sheet may be reduced. Thus, an addition amount thereof should be significantly suppressed as much as possible.

Nitrogen (N) is an element, inevitably contained during the production, so an addition range of N is limited to 0.1% or less (including 0%).

Titanium (Ti) is a strong carbide forming element, combined with carbon to form a carbide. The carbide formed at this time is an element effective in refining a grain size by inhibiting crystal grain growth. Moreover, when Ti is added in combination with boron, a high temperature compound is formed in a columnar-grained boundary to prevent grain boundary cracking from occurring. In addition, Ti has a scavenging effect in which a fraction of each of C and N is lowered by forming a compound with C and N. Thus, Ti is an essential element for improving damping capabilities. However, if an addition amount of Ti exceeds 1.00%, an excessive amount of Ti may be segregated in a crystal grain boundary and grain boundary embrittlement may be caused, or a precipitation phase may be excessively coarse. Thus, a grain growth effect may be lowered. Therefore, the addition amount of Ti is limited to being 1.0% or less.

The high Mn steel sheet according to another aspect to the present disclosure additionally includes one, two, or more among 0 wt% to 3 wt% of silicon (Si), 0.005 wt% to 5.0 wt% of chromium (Cr), 0.005 wt% to 2.0 wt% of nickel (Ni), 0.005 wt% to 0.5 wt% of niobium (Nb), 0.0001 wt% to 0.01 wt% of boron (B), 0.005 wt% to 0.5 wt% of vanadium (V), and 0.005 wt% to 1 wt% of tungsten (W).

Silicon (Si) is a solid solution strengthening element, and is an element for increasing yield strength by reducing a grain size by a solid solution effect. Thus, Si is necessary to secure strength. However, if an addition amount of Si is increased, during hot rolling, silicon oxide is formed on a surface of a steel sheet. Thus, pickling properties are deteriorated, so surface qualities of a steel sheet may be deteriorated, as a disadvantage. Moreover, due to addition of a large amount of Si, the weldability of steel may be significantly lowered. Thus, an upper limit of the addition amount of Si is limited to 3%.

Chromium (Cr) reacts with external oxygen during a hot rolling or annealing operation, and a Cr-based oxide film (Cr₂O₃) having a thickness of 20 µm to 50 µm is preferentially formed on a surface of a steel sheet, so Mn and Si, contained in the steel, are prevented from being eluted into a surface layer. Thus, Cr may act as an element for contributing to stabilization of a structure of a surface layer and improving plating surface properties.

However, if Cr is included in an amount less than 0.005%, the effect described above is insignificant. If Cr is included in an amount exceeding 5.0%, chromium carbide is formed, so workability and delayed fracture properties are deteriorated. Thus, an upper limit of the content of Cr is limited to 5.0%.

Nickel (Ni) contributes to the stabilization of the austenite, which is not only advantageous for improving the elongation but also contributing effectively to the high temperature ductility. If the content of Ni, a strong high temperature toughness improving element, is less than 0.005%, an effect on high temperature toughness is insignificant. If an added content of Ni increases, Ni has a significant effect on prevention of delayed fracture and slab cracking. However, material costs may be high, so production costs may be increased. Thus, the content of Ni is Limited to 0.005% to 2.0%.

Niobium (Nb) is a carbide forming element for forming carbide by being combined with carbon in the steel. In the present disclosure, Nb may be added for the purpose of increasing the strength and refining the grain size. According to the related art, Nb forms a precipitate at a lower temperature as compared to Ti, so Nb is an element having significant effects of refining a crystal grain size and strengthening precipitation by formation of a precipitate. Thus, Nb may be added in an amount of 0.005% to 0.5%. However, if an addition amount of Nb is less than 0.005%, the effect described above is insignificant. On the other hand, if Nb is added in an amount exceeding 0.5%, an excessive amount of Nb is segregated in a grain boundary, thereby causing grain boundary embrittlement, or a precipitate may be excessively coarse, thereby lowering a growth effect of a crystal grain. Moreover, in a hot rolling process, recrystallization is delayed, so rolling load may be increased. Thus, the addition amount of Nb is Limited to 0.005% to 0.5%.

Vanadium (V) and tungsten (W) are elements for forming carbonitride by being combined with C and N together with Ti. In the present disclosure, since a fine precipitate is formed at a low temperature, a precipitation strengthening effect may be obtained. Moreover, V and W may be important elements for securing austenite. However, if two elements are added in small amounts, less than 0.005%, the effect described above is insignificant. On the other hand, if V is added in an amount exceeding 0.5% and W is added in an amount exceeding 1.0%, a precipitate is excessively coarse, so a grain growth effect may be lowered, which may cause hot brittleness. Thus, the addition amount of V is Limited to 0.005% to 0.5%, while the addition amount of W is limited to 0.005% to 1%.

Boron (B) is added with Ti, and thus a high-temperature compound is formed in a grain boundary, so grain boundary cracking may be prevented. However, if B is added in a small amount of 0.0001% or less, there may be no effect. If B is added in an amount of 0.01%, a boron compound is formed, so surface properties may be deteriorated. Thus, a range of B is limited to 0.0001% to 0.01%.

Hereinafter, a method for manufacturing a high Mn steel sheet having excellent damping properties will be described.

In the method for manufacturing a high Mn steel sheet according to the present disclosure, steel, which has the composition and composition range, and in which a microstructure is comprised of a austenite as main phase, is heated at a heating rate of 0.01°C/s to 200°C/s, and maintained at a heat treatment temperature of Ac1°C to Ac3+50°C for 0.01 second to 24 hours, and is then cooled to room temperature at a cooling rate of 0.01°C/s or more.

The high Mn steel sheet may be a cold rolled steel sheet or a hot rolled steel sheet.

The microstructure of the high Mn steel sheet consists of epsilon martensite and austenite.

In the heating, if a heating rate exceeds 200°C/s, Ac1 and Ac3 temperatures are raised. Thus, even when heat treatment is performed in the range of the present disclosure, there is a problem in which an average particle diameter of a microstructure exceeds 2 µm. Therefore, an upper limit of a heating rate is limited to 200°C/s. If the heating rate is 0.01°C/s or less, during an operation, coarse carbides may be generated due to phase instability. Therefore, the heat treatment should be performed at a rate of 0.01°C/s or more.

If the heat treatment is performed at a temperature less than Ac1, transformation does not proceed, so there may be a problem in which a heat treatment effect can not be obtained. If a heat treatment temperature exceeds Ac3+50°C, there may be a problem in which an average particle diameter of a microstructure exceeds 2 µm. Thus, the heat treatment temperature is limited to Ac1°C to Ac3+50°C.

If the heat treatment time is less than 0.01 second, the application of recrystallization and recovery is insignificant, so an effect of heat treatment may be not obtained. If the heat treatment time exceeds 24 hours, there may be a problem in a process in which excessive oxidation occurs, so base iron is removed, and excessive heat treatment costs are consumed, as well as a problem in a microstructure in which a microstructure significantly grows, so an average particle diameter thereof is greater than a target particle diameter.

If the cooling is performed at a cooling rate less than 0.01°C/s, there may be problems in which an average particle diameter of a microstructure is increased during the cooling, and coarse carbides are generated due to phase instability. Thus, a lower limit of a cooling rate is limited to 0.01°C/s. There is no upper limit of a cooling rate. As the cooling rate is increased, it may be more advantageous to secure epsilon martensite and secure a fine average particle size.

### [Mode for Invention]

Hereinafter, an Example of the present disclosure will be described in detail. The following example is for the purpose of understanding the present disclosure and is not intended to limit the present disclosure.

A cold rolled steel sheet, including 0.02 wt% of C, 17 wt% of Mn, 0.01 wt% of N, 0.008 wt% of P, 0.008 wt% of S, 0.03 wt% of Ti, and Fe and inevitable impurities, was heated at a heating rate of 5°C/s, and was then maintained for the heat treatment time at a heat treatment temperature illustrated in Table 1. Then, the heat treated steel sheet was cooled to room temperature at a cooling rate of 5°C/s.

Regarding the steel sheet, having been heat-treated and cooled, an average particle diameter of a microstructure and the fraction of epsilon martensite were investigated, and a result thereof is illustrated in Table 1 and FIG. 1.

**[Table 1]**

| Classificati on | Heat Treatment Temperature (°C) | Heat Treatment Time (min) | Particle Diameter (µm) | Area Fraction (%) of Epsilon Martensite |
|---|---|---|---|---|
| Example | 600 | 30 | 1.23 | 6.2 |
| Comparative Example 2 | 800 | 30 | 3.6 | 14.9 |
| Comparative Example 3 | 900 | 10 | 6.7 | 16.8 |
| Comparative Example 4 | 1000 | 30 | 6.7 | 34.6 |

As disclosed in Table 1 and FIG. 1, the Example, heat treated at 600°C, is compared with the Comparative Examples (2 to 4), heat treated at 800°C to 1000°C. In the case of Comparative Examples (2 to 4) in which heat treatment temperatures were 800°C, 900°C, and 1000°C, respectively, the area fraction of epsilon martensite was greater, as compared to the Example, heat treated at 600°C. However, a particle diameter of the Example, heat treated at 600°C, was smaller than a particle diameter of the Comparative Examples (2 to 4), heat treated at 800°C to 1000°C.

Meanwhile, in the case of Example, heat treated at 600°C according to the present disclosure, an average particle diameter of a microstructure was 2 µm or less.

FIG. 2 is a drawing illustrating a dilatometer cycle of heat treatment illustrated in FIG. 1.

In FIG. 2, Ac1 and Ac3 are confirmed, and the Example is a result in which a heat treatment was performed at Ac3 + 30°C.

In FIG. 3, the Example, heat treated at 600°C, and Comparative Example (4), heat treated at 1000°C, were measured using a friction coefficient method. A result of measuring Specific Damping Capacity (SDC) is illustrated therein.

Here, SDC indicates the damping capacity (a property in which an object absorbs vibrations).

Referring to FIGS. 1 and 3, a room temperature SDC value of damping steel having a microstructure according to the Example, heat treated at 600°C, is a value 2.5 times that of damping steel according to Comparative Example (4). In other words, a SDC value of Example, heat treated at 600°C, is 0.00025, and a SDC value of Comparative Example (4), heat treated at 1000°C, was measured as 0.0001.

The area fraction of epsilon martensite of the Example, heat treated at 600°C, was relatively low. However, a particle diameter thereof was small, so a structure may be finely and uniformly distributed. In this case, when a steel sheet, in which residual dislocation and an interface together with epsilon martensite are present, was affected by an external shock, a rate of conversion from energy to thermal energy was increased. Thus, damping capacity is improved, so damping properties may be excellent.

According to the related art, when a room temperature SDC value is 0.00015 or more, damping properties are excellent.

Through comprehensive results, when heat treatment is performed according to the present disclosure, an average particle diameter of 2 µm or less is secured. Thus, it can be seen that excellent damping properties may be secured.

In the case of the Comparative Examples the area fraction of epsilon martensite is high, as compared to the Example. On the other hand, an average particle diameter of a microstructure is great. Thus, the damping performance is inferior.

## Claims

1. A high Mn steel sheet having excellent damping properties, comprising
0.1 wt% or less of carbon (C), 8 wt% to 30 wt% of manganese (Mn), 0.1 wt% or less of phosphorus (P), 0.02 wt% or less of sulfur (S), 0.1 wt% or less of nitrogen (N), 0 wt% to 1.0 wt% of titanium (Ti), the balance of Fe and inevitable impurities, the high Mn steel sheet further optionally comprising one, two, or more among 0 wt% to 3 wt% of silicon (Si), 0.005 wt% to 5.0 wt% of chromium (Cr), 0.005 wt% to 2.0 wt% of nickel (Ni), 0.005 wt% to 0.5 wt% of niobium (Nb), 0.0001 wt% to 0.01 wt% of boron (B), 0.005 wt% to 0.5 wt% of vanadium (V), and 0.005 wt% to 1 wt% of tungsten (W),
a microstructure of the steel sheet consists of epsilon martensite and austenite, and an average particle diameter of each of the epsilon martensite and the austenite is 2 µm or less .

2. The high Mn steel sheet having excellent damping properties of claim 1, wherein a room temperature specific damping capacity value of the steel sheet is 0.00015 or more.

3. A method for manufacturing a high Mn steel sheet of claim 1, comprising:
heating a high Mn steel sheet, including 0.1 wt% or less of carbon (C), 8 wt% to 30 wt% of manganese (Mn), 0.1 wt% or less of phosphorus (P), 0.02 wt% or less of sulfur (S), 0.1 wt% or less of nitrogen (N), 0 wt% to 1.0 wt% of titanium (Ti), the balance of Fe and inevitable impurities, the high Mn steel sheet further optionally comprising one, two, or more among 0 wt% to 3 wt% of silicon (Si), 0.005 wt% to 5.0 wt% of chromium (Cr), 0.005 wt% to 2.0 wt% of nickel (Ni), 0.005 wt% to 0.5 wt% of niobium (Nb), 0.0001 wt% to 0.01 wt% of boron (B), 0.005 wt% to 0.5 wt% of vanadium (V), and 0.005 wt% to 1 wt% of tungsten (W), to a heat treatment temperature of Ac1°C to Ac3+50°C at a heating rate of 0.01°C/s to 200°C/s;
maintaining the high Mn steel sheet for 0.01 second to 24 hours at the heat treatment temperature; and
cooling the high Mn steel sheet to room temperature at a cooling rate of 0.01 °C/s or more.

4. The method for manufacturing high Mn steel sheet having excellent damping properties of claim 3, wherein a microstructure of the high Mn steel sheet consists of epsilon martensite and austenite.

## Patentansprüche

1. Hoch manganhaltiges Stahlblech mit ausgezeichneten Dämpfungseigenschaften, umfassend:
0,1 Gew.-% oder weniger an Kohlenstoff (C), 8 Gew.-% bis 30 Gew.-% an Mangan (Mn), 0,1 Gew.-% oder weniger an Phosphor (P), 0,02 Gew.-% oder weniger an Schwefel (S), 0,1 Gew.% oder weniger an Stickstoff (N), 0 Gew.-% bis 1,0 Gew.-% an Titan (Ti), wobei es sich bei dem Rest um Fe und unvermeidbare Verunreinigungen handelt, wobei das hoch manganhaltige Stahlblech darüber hinaus optional ein, zwei oder mehr Element/e, darunter 0 Gew.-% bis 3 Gew.-% an Silicium (Si), 0,005 Gew.-% bis 5,0 Gew.-% an Chrom (Cr), 0,005 Gew.-% bis 2,0 Gew.-% an Nickel (Ni), 0,005 Gew.-% bis 0,5 Gew.-% an Niob (Nb), 0,0001 Gew.-% bis 0,01 Gew.-% an Bor (B), 0,005 Gew.-% bis 0,5 Gew.-% an Vanadium (V) und 0,005 Gew.-% bis 1 Gew.-% an Wolfram (W) umfasst,
eine Mikrostruktur des Stahlblechs aus Epsilon-Martensit und Austenit besteht, und ein mittlerer Partikeldurchmesser jeweils des Epsilon-Martensits und Austenits 2 µm oder weniger beträgt.

2. Hoch manganhaltiges Stahlblech mit ausgezeichneten Dämpfungseigenschaften nach Anspruch 1, wobei ein raumtemperaturspezifischer Dämpfungskapazitätswert des Stahlblechs 0,00015 oder mehr beträgt.

3. Verfahren zum Herstellen eines hoch manganhaltigen Stahlblechs nach Anspruch 1, umfassend:
Erwärmen eines hoch manganhaltigen Stahlblechs, das 0,1 Gew.-% oder weniger an Kohlenstoff (C), 8 Gew.-% bis 30 Gew.-% an Mangan (Mn), 0,1 Gew.-% oder weniger an Phosphor (P), 0,02 Gew.-% oder weniger an Schwefel (S), 0,1 Gew.% oder weniger an Stickstoff (N), 0 Gew.-% bis 1,0 Gew.-% an Titan (Ti) enthält, wobei es sich bei dem Rest um Fe und unvermeidbare Verunreinigungen handelt, wobei das hoch manganhaltige Stahlblech darüber hinaus optional ein, zwei oder mehr Element/e, darunter 0 Gew.-% bis 3 Gew.-% an Silicium (Si), 0,005 Gew.-% bis 5,0 Gew.-% an Chrom (Cr), 0,005 Gew.-% bis 2,0 Gew.-% an Nickel (Ni), 0,005 Gew.-% bis 0,5 Gew.-% an Niob (Nb), 0,0001 Gew.-% bis 0,01 Gew.-% an Bor (B), 0,005 Gew.-% bis 0,5 Gew.-% an Vanadium (V) und 0,005 Gew.-% bis 1 Gew.-% an Wolfram (W) umfasst, auf eine Wärmebehandlungstemperatur von Ac1°C bis AC3+50°C mit einer Aufwärmrate von 0,01°C/s bis 200°C/s;
Halten des hoch manganhaltigen Stahlblechs für 0,01 Sekunden bis 24 Stunden auf der Wärmebehandlungstemperatur; und
Abkühlen des hoch manganhaltigen Stahlblechs auf Raumtemperatur mit einer Abkühlrate von 0,01°C/s oder mehr.

4. Verfahren zum Herstellen des hoch manganhaltigen Stahlblechs mit ausgezeichneten Dämpfungseigenschaften nach Anspruch 3, wobei eine Mikrostruktur des hoch manganhaltigen Stahlblechs aus Epsilon-Martensit und Austenit besteht.

## Revendications

1. Tôle d'acier à haut Mn ayant d'excellentes propriétés d'amortissement, comprenant
0,1 % en poids ou moins de carbone (C), 8 % en poids à 30 % en poids de manganèse (Mn), 0,1 % en poids ou moins de phosphore (P), 0,02 % en poids ou moins de soufre (S), 0,1 % en poids ou moins d'azote (N), 0 % en poids à 1,0 % en poids de titane (Ti), le solde de Fe et d'impuretés inévitables, la tôle d'acier à haut Mn comprenant en outre facultativement un, deux, ou plus de deux éléments parmi 0 % en poids à 3 % en poids de silicium (Si), 0,005 % en poids à 5,0 % en poids de chrome (Cr), 0,005 % en poids à 2,0 % en poids de nickel (Ni), 0,005 % en poids à 0,5 % en poids de niobium (Nb), 0,0001 % en poids à 0,1 % en poids de bore (B), 0,005 % en poids à 0,5 % en poids de vanadium (V), et 0,005 % en poids à 1 % en poids de tungstène (W),
une microstructure de la tôle d'acier étant composée de martensite epsilon et d'austénite, et un diamètre de particule moyen de chacune de la martensite epsilon et de l'austénite est de 2 µm ou moins.

2. La tôle d'acier à haut Mn ayant d'excellentes propriétés d'amortissement de la revendication 1, sachant qu'une valeur de capacité d'amortissement spécifique à température ambiante de la tôle d'acier est de 0,00015 ou plus.

3. Procédé de fabrication d'une tôle d'acier à haut Mn de la revendication 1, comprenant :
le chauffage d'une tôle d'acier à haut Mn, incluant 0,1 % en poids ou moins de carbone (C), 8 % en poids à 30 % en poids de manganèse (Mn), 0,1 % en poids ou moins de phosphore (P), 0,02 % en poids ou moins de soufre (S), 0,1 % en poids ou moins d'azote (N), 0 % en poids à 1,0 % en poids de titane (Ti), le solde de Fe et d'impuretés inévitables, la tôle d'acier à haut Mn comprenant en outre facultativement un, deux, ou plus de deux éléments parmi 0 % en poids à 3 % en poids de silicium (Si), 0,005 % en poids à 5,0 % en poids de chrome (Cr), 0,005 % en poids à 2,0 % en poids de nickel (Ni), 0,005 % en poids à 0,5 % en poids de niobium (Nb), 0,0001 % en poids à 0,1 % en poids de bore (B), 0,005 % en poids à 0,5 % en poids de vanadium (V), et 0,005 % en poids à 1 % en poids de tungstène (W), à une température de traitement thermique de Ac1 °C à Ac3+50 °C à une cadence de chauffage de 0,01 °C/s à 200 °C/s ;
le maintien de la tôle d'acier à haut Mn pendant 0,01 seconde à 24 heures à la température de traitement thermique ; et
le refroidissement de la tôle d'acier à haut Mn à température ambiante à une cadence de refroidissement de 0,01 °C/s ou plus.

4. Le procédé de fabrication d'une tôle d'acier à haut Mn ayant d'excellentes propriétés d'amortissement de la revendication 3, sachant qu'une microstructure de la tôle d'acier à haut Mn est composée de martensite epsilon et d'austénite.
